

# UNITED STATES PATENT OFFICE.

FRANK H. DAVIS, OF NEW YORK, N. Y., ASSIGNOR OF ONE-HALF TO FRANCIS R. COUGHLIN, OF NEW YORK, N. Y.

## FUSIBLE ADHERENT AND METHOD OF MAKING THE SAME.

1,374,492.

Specification of Letters Patent. Patented Apr. 12, 1921.

No Drawing.

Application filed February 4, 1919. Serial No. 274,856.

To all whom it may concern:

Be it known that I, FRANK H. DAVIS, a citizen of the United States, and residing at New York, in the county of Bronx and 5 State of New York, have invented certain new and useful Improvements in Fusible Adherents and Methods of Making the Same, of which the following is a specification, such as will enable those skilled in the 10 art to which it appertains to make and use the same.

This invention relates to fusible adherents used in securing gold leaf to strips, ribbons, tapes or sheets of paper or other protective material, or in the manufacture of 15 what is known as mounted or backed gold leaf which is usually made up into rolls of gold leaf tape, such as is shown, described and claimed in a prior patent granted to 20 Davis and Schumacher, Jan. 12, 1915, No. 1,124,869; and the object of this invention is to produce by an improved method a fusible adherent for securing gold leaf to the 25 paper strip or tape upon which it is mounted, which will possess all the required adhesive and fusible qualities of adherents of this class now in use but will be free of all 30 greasy or fatty substances that are now common in or forming part of fusible adherents thus eliminating shaded or dull appearances of the gold leaf when applied to a suitable backing strip due to the presence of 35 too much greasy or fatty substances in the fusible adherent employed; and a further object of the invention consists in an improved method of producing the desired adherent by treating a suitable product to produce by-products thereof, one of which is used in manufacturing said adherent while 40 the other of which may be diluted and used as a sizing for the gold leaf after it has been applied to, or mounted on, a suitable backing strip in the usual manner, and with these and other objects in view the invention consists in a fusible adherent of the 45 class and for the purpose specified, and in the method of producing it as hereinafter described and claimed.

My improved fusible adherent may be 50 made from what is known as white shellac, or the sap of various trees, such as the willow tree, or a by-product of these substances and in order to attain such by-product, I treat one of these substances, as for example, 55 white shellac by taking one quart of white

shellac to which is added two quarts of ammonia and one pound of table salt. These ingredients are placed in a suitable vat or container and boiled slowly for about seven hours, during which time water is added to 60 the solution at intervals to keep the same in a liquid state. After the above boiling operation is continued for a period of about two hours a dark substance will be noted on the top of the liquid, this substance is 65 shellac in a very thin and sticky state and is skinned off and placed in a suitable container and forms one of the by-products of the original white shellac employed and which is hereafter described. The above 70 described operation of skimming the sticky shellac from the top of the solution is repeated at about one-half to three-quarter hour intervals until but little of said substance appears on the top of the solution. 75

At the end of the period of about seven hours of slow boiling the solution, as above described, a hard substance or precipitate will be noticed in the bottom of the vat or container, this substance is the principal 80 product and is removed and allowed to thoroughly dry, after which it is crushed into the form of powder in any desired manner.

After attaining the principal product of 85 shellac in the form of a hard substance which is made into a powder as above described, I use said powder in forming or producing my improved fusible adherent in the following proportions:—3 ounces of the 90 principal product of shellac in powdered form; 1 gallon of benzin.

In producing the desired solution, the above proportions of the powdered product of shellac and benzin are placed in a suitable double boiler and heated until all of the solid or powdered substance has been thoroughly dissolved by the benzin, and this produces the fusible adherent which I use in attaching gold leaf to a strip or sheet of 95 suitable paper, and this product while having the required adhering qualities is free from all greasy or fatty substances which tend to discolor or effect the brightness of the gold leaf.

In the operation of applying or attaching gold leaf to one face of a strip or sheet of paper, the fusible adherent produced in the manner above described which is constantly 100 kept in a heated state, is applied to the face 110

of the strip or sheet of paper, after which the gold leaf is applied to the fusible adherent on said strip in the usual manner and is then allowed to dry.

- 5 I also preferably use the first named by-product of the shellac consisting of the thin sticky shellac substance, which is skimmed from the top of the shellac solution as a size or sizing by diluting it with a predetermined 10 amount of alcohol, and this solution is applied to the face of the gold leaf when the fusible adherent for connecting the same with a strip or sheet of paper is dried. From the foregoing it will be seen that both 15 the by-product and principal product are used in the manufacture of mounted or backed gold leaf, but it will also be understood that my invention is not limited to the use of the sticky shellac, above referred to, 20 as a sizing as any sizing that is now known, or in common use, may be employed, or milkweed sap in diluted form may be used for this purpose. While as above set out, I preferably employ one gallon of benzin in 25 connection with the powdered by-product of shellac for producing my fusible adherent, it will be understood that any highly volatile hydro-carbon product such as naphtha or gasolene might also be used for this purpose, but I have found in practice benzin gives the best results.

In the use of a strip or sheet of paper to one face of which gold leaf has been attached by my improved fusible adherent as well as 30 the shellac sizing formed by the by-product of shellac above set out, in the gold leafing of leather goods of various kinds and classes, paper, cloth or other surfaces, by the use of what is known as hot dies or stamps, the 35 gold leaf will be freed from the strip or sheet of paper to which it is attached by reason of the fusible adherent employed, and the sizing on the face of the gold leaf will be rendered plastic whereby the impressions of the die, or the figures thereof, will transfer corresponding impressions or figures of the gold leaf onto a suitable surface, and will adhere to said surface by the heated 40 sizing on said portions of gold leaf.

- 45 My invention is not limited to any specific method of transferring the gold leaf from a strip or sheet to which it is attached by my improved fusible adherent, as this may be performed in the usual or any desired manner, and while I have described one method 50 of producing a fusible adherent which will have all the desired qualities of adherents of the class specified but which is free from greasy or fatty substances, from one product 55 namely shellac, it will be understood that my invention is not limited to this specific method or product as I have found that some other resinous substance may be treated 60 to produce a product which would have the 65 desired adherent qualities as well as the

fusible qualities as the herein described fusible adherent, and again my invention is not limited to the specific proportions or amounts of the various ingredients employed in the production of my fusible adherent, and various changes in and modifications of these details of my invention may be made, within the scope of the appended claims, without departing from the spirit of my invention or sacrificing its advantages.

70 It will be observed that in the production of the fusible adherent herein described, I do not employ in connection therewith greasy or fatty substances, such as beeswax and similar material, but avoid the use of 80 this material as is clearly set out and for the purposes herein described.

Having fully described my invention, what I claim as new and desire to secure by Letters Patent, is:—

85 1. The herein described method of producing a fusible adherent which consists in first treating white shellac to obtain a principal product thereof by mixing one quart of shellac with two quarts of ammonia and one 90 pound of salt and boiling this solution until a hard product in the form of a sediment is obtained, separating said product from the solution, drying the same and then crushing it into powder form and mixing three 95 ounces of the powdered product of shellac with one gallon of benzin, substantially as described.

100 2. The herein described method of producing a fusible adherent and sizing used in the manufacture of mounted gold leaf which consists in first treating white shellac to obtain a by-product and principal product thereof by mixing one quart of shellac with two quarts of ammonia and one pound 105 of salt and boiling this solution to obtain a sticky liquid by-product which is used as a sizing and a solid product, separating the last named product from the solution, drying the same and grinding it into powdered form, and mixing three ounces of said powdered product of shellac with a gallon of benzin to form the fusible adherent.

110 3. The herein described method of producing a fusible adherent and sizing used in the manufacture of mounted gold leaf which consists in first treating white shellac to obtain a by-product and principal product thereof by mixing one quart of said shellac with two quarts of ammonia and one 115 pound of salt, boiling this solution to obtain a sticky liquid by-product which is used as a sizing and a solid product, separating the last named product from the solution, drying the same and grinding it into powdered form, mixing three ounces of said powdered product with a gallon of benzin to form the fusible adherent and diluting the first named liquid by-product of shellac in alcohol to form the desired sizing.

4. The herein described method of producing a fusible adherent adapted for use in the manufacture of mounted gold leaf, which consists in boiling shellac with a suitable solution of sodium chlorid in ammonia until a precipitate is formed on the bottom of the vessel and removing said precipitate, said precipitate when dried, crushed and dissolved in a suitable solvent forming said 10 fusible adherent.

5. The herein described method of producing a fusible adherent and size adapted for use in the manufacture of and use of mounted gold leaf which consists in boiling shellac with a solution of sodium chlorid in ammonia, removing from time to time the scum formed on the surface of the liquid and said scum when dissolved in a suitable solvent forming the said size, thereafter 15 continuing the boiling until a precipitate is formed on the bottom of the vessel and removing said precipitate, said precipitate when dried, crushed and dissolved in a suitable solvent forming the said fusible adherent. 20

25 6. The herein described method of producing a fusible adherent for use in the

manufacture of mounted gold leaf which consists in boiling shellac or equivalent resinous product with a solution of sodium chlorid in ammonia until a precipitate is formed in the bottom of the vessel, separating said precipitate from the solution, then drying, crushing and dissolving the same in a suitable solvent to form said fusible adherent. 30 35

7. A fusible adherent of the class described derived from shellac or equivalent resinous product by boiling said product with ammonium hydroxid and sodium chlorid solution until a precipitate is 40 formed, free from greasy or fatty substances and having fusible properties suitable for transferring gold leaf from its backing to the object upon which it is to be attached without discoloration of said gold leaf. 45

In testimony that I claim the foregoing as my invention I have signed my name in presence of the subscribing witnesses this 3rd day of February, 1919.

FRANK H. DAVIS.

Witnesses:

C. E. MULREANY,  
H. E. THOMPSON.